

# UNITED STATES PATENT OFFICE.

JOHN K. TULLIS, OF NEW YORK, N. Y., ASSIGNOR TO FULCRA TAN COMPANY, OF NEW YORK, N. Y., A CORPORATION OF DELAWARE.

## TANNING.

1,390,735.

Specification of Letters Patent. Patented Sept. 13, 1921.

No Drawing.

Application filed September 24, 1918. Serial No. 255,477.

To all whom it may concern:

Be it known that I, JOHN K. TULLIS, a subject of the King of Great Britain, and a resident of New York city, in the county of 5 New York and State of New York, have invented certain new and useful Improvements in Tanning, of which the following is a specification.

This invention relates to tanning; and it 10 comprises a combined process of tanning wherein hide is first treated with a material containing chromic acid ( $\text{CrO}_3$ ) such as a chromate or bichromate to give a light impregnation and is thereafter treated with a 15 sulfite waste liquor preparation or solution, having its normal constituents substantially unaltered thereby reducing the chromic acid to the state of sesquioxid of chromium or and advantageously to that of a chromate 20 of chromium, said sulfite waste liquor also effecting a tanning action; all as more fully hereinafter set forth and as claimed.

It is of course well known in the art to tan hides with various chrome compounds. 25 In one way of tanning, the hide is treated with a solution containing a salt of the sesquioxid of chromium ( $\text{Cr}_2\text{O}_3$ ), such as a solution containing chrome alum together with other bodies, salts of chromium sesquioxid combined with weak acids, etc. In another method of tanning the hides are treated with a bichromate, such as potassium bichromate or sodium bichromate and thereafter with a reducing agent capable of 30 converting chromium trioxid ( $\text{CrO}_3$ ) into the sesquioxid, this agent being usually a mineral salt such as a hyposulfite, a sulfite, etc. In the present method of tanning I use a bichromate but instead of employing a 35 special mineral salt to reduce the chromium trioxid or chromic acid to the sesquioxid I employ a body which itself has a tanning effect, namely a material containing the characteristic organic solids of sulfite waste liquor in a substantially unaltered state. 40 Unlike most tanning materials now in use, various preparations made from sulfite waste liquor have the property of converting chromic acid contained in a hide into a condition in which it will tan; that is of reducing it. The reduction by sulfite waste liquor may go so far as to convert the chromic acid compounds into compounds of chromium sesquioxid or it may be stopped at a 45 point short of this; a point where part of

the chromium trioxid is reduced and the rest remains as such. The result of this is to produce a chromate of chromium in the hide. The chromates of chromium are brown bodies which have, as I have found, a good 50 tanning effect and are useful in accelerating and aiding subsequent tanning with other bodies. Where the reduction of the bichromate goes so far as to produce sesquioxid of chromium, the hide is left, at this stage, 55 with a bluish or greenish tinge but where the reduction is only partial and a chromate of chromium is formed in the hide, the color is brownish.

In the manufacture of paper pulp by the 60 sulfite process, wood is digested under pressure with a solution of calcium (or calcium and magnesium) bisulfite. In the digestion various reactions go on by virtue of which about one-half the wood, the so-called "lignone", goes into solution by uniting with the acid sulfite to form new soluble organic bodies. The rest of the wood, the cellulose, remains undissolved as ordinary paper pulp. For the sake of a name, 65 the bodies found in the solution, the "sulfite waste liquor" are often termed lignosulfonates. Where the original sulfite liquor is a solution of acid sulfite of calcium, the waste sulfite liquor is regarded as a solution 70 of lignosulfonates of calcium. Where, as is often the case, the original sulfite liquor contains both magnesium and calcium acid sulfites, the characteristic bodies of the waste sulfite liquor are regarded as a mixture of 75 magnesium and calcium lignosulfonates. As the liquor leaves the digester it is rather weak and somewhat acid; containing a small fraction of a per cent. of unchanged sulfuric acid or acid sulfite. The acidity is 80 not great but some acidity exists. As a rule this liquid is not of a concentrated nature, containing only a few per cent. of solid matter. Its density may be from 3 to 5° or 6° Baumé. From this liquid various tanning 85 preparations can be made. One such preparation which finds extensive sale on the market is made by simply neutralizing the raw liquor and evaporating *in vacuo* to a rather high density, usually around 30° 90 Baumé, (Patent 833,634), this giving a solution of the essential substances of waste sulfite liquor chemically unchanged. Alone, the raw sulfite liquor is not readily concentrated by heat without far-going decomposi- 95 100 105 110

tion and loss of tanning bodies but if preliminarily somewhat neutralized it may be readily evaporated without substantial loss of valuable constituents. Other tanning preparations are made from the concentrated liquor so prepared by treating it with a sulfate of a sesquioxid having tanning properties, that is sulfate of iron, sulfate of alumina or sulfate of chromium. The lignosulfate of lime by double decomposition gives insoluble sulfate of lime which precipitates and a soluble lignosulfate of iron, aluminum or chromium as the case may be. These preparations are usually somewhat acid to litmus and do not give precipitates with metal salts. Other tanning preparations are made by treating the raw liquor with a little sulfuric acid and bisulfate of soda, thereby removing the lime as sulfate and leaving a liquid containing lignosulfonic acid.

In the present invention a hide after the usual beam house preparation is first given a light impregnation with a solution of a bichromate. Either the bichromate of potassium or bichromate of sodium may be used, although I find the latter more advantageous for several reasons. Chromic acid ( $\text{CrO}_3$ ) may be used but is ordinarily more expensive. In order to assist the penetration of the bichromate into the hide it is useful to employ a little aluminum sulfate and magnesium sulfate (Epsom salts) in the solution. A desirable bath for the present purposes may be made by dissolving sodium bichromate in water to give a solution of about 1 per cent.; a strength sufficient to give a light impregnation. In this solution may be dissolved 2 per cent. of aluminum sulfate and 3 per cent. of Epsom salts. The hide is immersed in or wetted with the bichromate solution for a length of time sufficient to secure good penetration; ordinarily two or three days. It is then removed from the chrome solution and treated with a slightly acid sulfite waste liquor preparation for four or five days. The greater the acidity the further the reduction of the chromium will go. I prefer a degree of acidity of say 0.6 or 0.7 per cent., as this causes only a partial reduction, forming chromate or chromium instead of reducing to sesquioxid. In addition to re-

ducing the chromium the solution of the sulfite waste liquor also tans. I therefore obtain what may be called a combination tanning; a tanning by reduced chromium (as chromium sesquioxid or as chromate of chromium) and a tanning by the sulfite waste liquor. If the leather is to be for harness and like purposes no further tanning may be necessary. If it is to be used for sole leather or similar purposes, I find it best to follow with another tanning operation. For this final tanning I may use a strong waste sulfite liquor such as the commercial 30° Baumé preparations or another tanning material. Various mixtures of concentrated waste sulfite liquor with other tanning material, such as oak, quebracho, mangrove, chestnut, etc., may be employed.

What I claim is:—

1. The process of tanning which comprises treating a hide with a solution of bichromate to produce a light impregnation and then effecting reduction of chromic acid to chromate of chromium in the hide and tanning by treating with a sulfite waste liquor material containing its normal constituents substantially unchanged.

2. The process of tanning which comprises treating a hide with a solution of bichromate containing aluminum sulfate and magnesium sulfate, and then effecting reduction in the hide and tanning by treating with a sulfite waste liquor material.

3. The process of tanning which comprises lightly impregnating a hide with bichromate, then reducing in the hide and tanning with a sulfite waste liquor material containing its normal constituents substantially unchanged, and effecting a further tanning with a tanning extract.

4. The process of tanning which comprises lightly impregnating a hide with bichromate, then reducing chromic acid to chromate of chromium in the hide and tanning with a sulfite waste liquor material, and effecting a further tanning with a tanning extract comprising a waste sulfite liquor preparation.

In testimony whereof, I affix my signature hereto.

JOHN K. TULLIS.

**Certificate of Correction.**

It is hereby certified that in Letters Patent No. 1,390,735, granted September 13, 1921, upon the application of John K. Tullis, of New York, N. Y., for an improvement in "Tanning," errors appear in the printed specification requiring correction as follows: Page 2, line 85, claim 2, after the word "material" and before the period insert the phrase *containing its normal constituents substantially unchanged*; same page, line 97, claim 4, after the word "material" and before the comma insert the phrase *containing its normal constituents substantially unchanged*; and that the said Letters Patent should be read with these corrections therein that the same may conform to the record of the case in the Patent Office.

Signed and sealed this 16th day of May, A. D., 1922.

[SEAL.]

**KARL FENNING,**  
*Acting Commissioner of Patents.*